

Oct. 18, 1938.

W. E. MOORE ET AL

2,133,329

METHOD FOR HEAT TREATING FURNACE LININGS

Filed Sept. 1, 1936

3 Sheets-Sheet 1



Oct. 18, 1938.

W. E. MOORE ET AL

2,133,329

## METHOD FOR HEAT TREATING FURNACE LININGS

Filed Sept. 1, 1936

3 Sheets-Sheet 2



INVENTORS

25 William E. Moore and  
William S. Wallis  
by their atto's  
Stubbins, Glenbo & Carmelee

Oct. 18, 1938.

W. E. MOORE ET AL

2,133,329

METHOD FOR HEAT TREATING FURNACE LININGS

Filed Sept. 1, 1936

3 Sheets-Sheet 3



## UNITED STATES PATENT OFFICE

2,133,329

## METHOD FOR HEAT TREATING FURNACE LININGS

William E. Moore, Pittsburgh, Pa., and William B. Wallis, New York, N. Y., assignors to Pittsburgh Research Corporation, Pittsburgh, Pa., a corporation of Delaware

Application September 1, 1936, Serial No. 98,918

2 Claims. (Cl. 13—35)

Our invention relates in general to refractory furnace linings and to the art of heat treating them, and more particularly to methods for burning in the refractory linings of furnaces and like structures and to a lining formed in situ.

Furnaces such as are used for melting, refining or treating metals, glass, or the like, or furnaces for boilers and the like are subject to relatively high temperatures and are usually constructed with highly refractory linings. These linings are commonly made from firebrick aggregates of silica or magnesite sand and the like, cemented or bonded together by a binder, such as, for example, fireclay or hydrocarbons and similar substances. The fusing or maturing point of the binders employed is much lower than that of the refractory material from which the linings and particularly the bottoms are formed, and the use of such a binder impairs the effectiveness of the refractory material in direct proportion to the amount of binder used, as it renders the furnace linings more readily fusible at lower temperatures and more susceptible to disintegration. In the repairs of such furnaces, refractory substances with a binding material such as we mentioned, are usually employed and are subject to the same objections.

It is also desirable that the lining have as dense and as homogeneous a surface as possible, so that the content of the furnace, such as molten metal, may not find its way into the body of the lining as the deterioration of the lining depends upon the extent of surface exposed to the corrosive action of the molten charge and the more porous the lining, the greater is the surface exposed. It is, therefore, a great advantage to fuse the lining of the furnace, particularly those parts which come into contact with highly heated metals or highly heated or corrosive products of combustion and to fuse such portions without the use of binders or fluxes which will impair the resistance of the lining material to high temperatures and corrosion.

Heretofore, attempts have been made to burn in the bottoms of electric furnaces having highly refractory bottoms made from materials, such as magnesite, by means of the ordinary electric arc which is generally set up to arc against a delta or T made of carbon electrodes placed across the bottom. While this plan may have some advantages for small furnaces, it becomes less practical as the size of the furnace increases and, even with small furnaces, it has heretofore been essential to reduce the melting temperature of a highly refractory material, such as magnesite, by adding to it a flux such as 8 to 10% of open hearth

slag or silica, etc. The same difficulty applies to highly refractory bottoms and linings in open hearth furnaces and the like, as the heat is not available there from combustion of fuel to burn in highly refractory bottoms. Even with such heat as is available, great damage resulting from the overheating thereof is usually done to the roof and other parts of the refractory lining of the furnace when burning in the bottom so that in open hearth furnaces the life of the refractory lining is still further sacrificed by fluxing it more liberally.

The desirable condition, for example, in a metal melting furnace bottom and lining exposed to the action of molten metals and slag, is to have the inner layers thereof thoroughly fused together into a vitreous mass without the use of fluxes or binders. The heat resisting properties of the refractory material need not therefore be impaired by adulteration with fluxes, and we have found that such linings made according to our invention very successfully resist the dissolving action of slag and the boiling action of molten metal and like sources of lining deterioration.

The electric arc has a temperature sufficiently high to melt any known refractory material if the arc be concentrated or blown directly against the material. By means of our invention, we have provided a method and apparatus which utilizes the properties of the electric arc for burning in or fusing the refractory linings, particularly the bottoms, banks or side walls, on all kinds of furnaces, electric, open hearth, or other kinds, but without overheating of other parts of the furnace structure. Furthermore, it is thus possible to provide a lining which is made from unfluxed refractory material which may be formed in situ and fused to the shape of the furnace or like structure. The refractory material may be preformed, if desired, or a loose or granular material of any size particle may be employed, such as granular magnesite. Our device consists of a portable apparatus having supports for two electrodes of suitable material such as carbon or graphite inclinably mounted like a V with the arcing points nearest the bottom of the V. By means of this arrangement, the arc is blown or repelled vigorously by magnetic repulsion away from the bottom of the V and may be directed against the material to be fused or sintered in. The device is portable and is arranged for manipulation of the electrodes to different positions so that the arc may be brought to bear on practically any desired part of the furnace lining and thus fuse the refractory material progressively until the de-

5

10

15

20

25

30

35

40

45

50

55

sired portions of the furnace lining are covered with a vitreous mass or to use the expression of the industry "burned in".

By our invention, we provide a simple and convenient arrangement whereby an electric arc can be maintained between the electrodes of a portable apparatus which can be readily manipulated so that the heat therefrom may be directed against any desired point.

10 In the accompanying drawings, illustrating present preferred embodiments of our invention, and in which like numerals are employed to designate like parts throughout the same;

15 Figure 1 is an elevation showing our device in position in a furnace;

Figure 2 is a view, partly in section, through one of the holders and to a larger scale than Figure 1;

20 Figure 3 is a view along the section III-III of Figure 2;

Figure 4 is a view along the section IV-IV of Figure 2;

25 Figure 5 is a plan view of the electrode end of the apparatus.

Figure 6 is an elevation of the outer end of the control end of the apparatus;

25 Figures 7, 8, and 9 are detail views of portions of the apparatus.

In the drawings, we have shown in Figure 1 a portable water-cooled electric torch  $T$  made according to our invention in position to burn in the bottom  $B$  of furnace  $F$ . It is to be understood that the apparatus is suitable not only for burning in the refractory bottom but by proper manipulation other parts of the lining as well, which are made of refractory material, may be treated.

The torch consists of two copper electrode holders  $10$ , each mounted on an electrode carrying member or arm  $11$ . Each of the electrode arms  $11$  are slidably and rotatably mounted within a copper contact sleeve  $12$ , to which a suitable terminal  $13$  for the electric power supply is attached. Adjacent the holder end of the arms  $11$  is a metal spacing member  $14$  having ends which embrace an insulated sleeve  $15$ , each sleeve surrounding the arm  $11$  in such manner that each of the arms  $11$  may be rotated within its associated sleeve. At the outer end of the electrode arms  $11$ , that is the end distant from the electrode holders  $10$ , suitable adjusting handles  $16$  are secured. By means of these handles, which are made of insulating material such as wood, fibre, or synthetic resin, etc., the electrode arms can be moved longitudinally and rotated, and the apparatus as a whole can be manipulated. Fixedly mounted on each electrode arm  $11$ , between the handle  $16$  and contact sleeve  $12$  is a rock crank  $17$ . The cranks  $17$  are swivelly connected by an insulating connecting link  $18$ , preferably made of bakelite, fibre, or other physically strong insulating material, so that when one arm is rotated in one direction, the other arm will move simultaneously in the opposite direction and in the same amount. The ends of arm  $11$  adjacent the handles  $16$  are rotatably secured together by a spacing link  $19$  of insulating material.

The electrode arm  $11$  is preferably made from hollow copper tubing and is attached to the holder  $10$ , in any suitable manner, as, for example, by screw threading. The holder  $10$  has an internal water passage  $20$  therearound and to one end of this water passage a pipe  $21$  is attached.

75 This pipe is smaller in diameter than the inside

diameter of the electrode arm  $11$ , and passes therethrough, so that there is an annular space between the pipe  $21$  and the inner wall of arm  $11$ , into which space the other end of passage  $20$  leads. Pipe  $21$  extends through the disc  $22$  which closes the handle end of the electrode arm  $11$  and has a connection  $23$  to a suitable source of water supply (not shown). Cooling water may thus be passed through pipe  $21$  around passage  $20$  in holder  $10$ , back through the annular space between the electrode arm and tube  $21$  and discharged through discharge connection  $24$ .

Contact sleeves  $12$  are each mounted against movement within an insulating sleeve  $25$ , which is received in a spacing member or support  $26$ . The spacing member consists of an upper portion  $27$  and a lower portion  $28$ , removably secured together. The ends of both of these portions are shaped to embrace and retain insulating sleeve  $25$  in a predetermined position. A lifting hook  $29$  is secured to arm spacing member  $26$ . The lower portion  $28$  has a rearwardly projecting horizontal arm  $30$  and a downwardly projecting bifurcated portion  $31$  which is pivotally secured by bolt  $32$  to the head  $33$  of a hollow screw-threaded upright or support  $34$ , which is adjustably fastened to movable truck  $35$ .

Truck  $35$  has two front wheels  $36$  and a swivel wheel  $37$  at the rear supporting a framework  $38$  through which the hollow upright  $34$  projects and is supported on the frame  $38$  by adjusting nut  $39$ , which is in anti-friction engagement therewith. By manipulation of nut  $39$ , the apparatus as a whole may be adjusted to the desired vertical position. A suitable counterweight  $40$  may be placed, if necessary, on frame  $38$  to resist the turning movement due to the counterbalance device hereinafter to be described.

In order to counterbalance the weight of the electrode-holders and electrodes so that the apparatus may be readily worked by man power, we provide a counterbalance device. This device consists of a balance arm  $41$  having an upwardly inclined reduced end portion which is received in an opening  $42$  in supporting member  $34$ . The arm has various holes  $43$  along its length into any one of which, one end of a suitable spring  $44$  may be secured. The other end of spring  $44$  is fastened to hook member  $45$  which, in turn, is attached to horizontal arm  $30$  by an adjustable screw-threaded connection  $46$ . By placing one end of spring  $44$  in a suitable hole in balance arm  $41$ , the other end in hook member  $45$ , which, in turn, is secured in a suitable position to arm  $30$ , and by adjusting the connection  $46$ , the proper counterbalancing force may be secured. In some installations, counterbalancing may be secured by means of suitably insulated counterweights (not shown) connected to arms  $11$ .

When placing the apparatus in position and at other times during the operation of the apparatus, it may be desirable to move the torch itself and the truck  $35$  as a unit. To prevent the torch  $T$  from swinging in a horizontal plane with respect to the truck  $35$ , we provide a lock member or latch  $47$  which is pivotally secured to the bifurcated portion  $31$  of spacing member  $26$  so that when the torch is to be locked to truck  $35$ , latch  $47$  will be in the position shown in Figures 1, 2 and 9, where the depending portion of the latch is received in groove  $48$  formed in the framework  $38$ . Secured to member  $47$  is a hook  $49$ , which when connected to spacing member  $26$ , will hold latch  $47$  out of engagement with groove  $48$  and thus permit the torch to freely 75

swivel on the truck 35. In Figure 2, the latch 47 is shown in dotted lines out of locking engagement.

The electrodes 50 of a suitable size and formed 5 from a suitable material such as carbon or graphite, are secured in the electrode holder or clamp 10 by any suitable means such as clamping wedges 51, preferably made of copper, which are driven in from the upper side of the holder.

10 *Operation of the apparatus*

A layer of refractory material is rammed in 15 on the elementary bottom layers of the furnace lining which are usually of brick. The electrode end of the torch is projected through a door or other suitable opening into the furnace and the water cooling circulation is established. An arc 20 is then struck by rocking the arms 11 by means of handle 16 until the tips of the electrodes 50 contact, after which they are rocked back slightly to draw the arc to the desired length, whereupon the free-burning arc is blown or projected 25 against the lining at the desired point until the refractory lining is burned in or sintered. The arc is then moved from place to place on the 30 lining until the desired area is burned in or sintered. Due to the construction of the torch, the arms may be moved backwards or forward tilted and rotated, and the truck may be manipulated so that all the desired area of the furnace lining may be processed.

It is also possible to disconnect the torch from the truck by removing bolt 32. The torch may then be suspended by means of hook 29 from an 35 overhead crane or the like, or from a convenient part of the structure to be treated, in which circumstances, the electrode end of the torch may be inserted into the furnace by first removing the roof or it may be introduced through any other convenient opening. In case the torch is 40 suspended from a convenient support, the rock cranks 17 may be adjusted in position along the arms, so that sliding movement of the arms in the contact sleeves 21 is restricted. Many modern furnaces, especially electric furnaces, are of 45 the tilting type and have removable roofs and

the overhead suspension of the torch is particularly applicable when treating such furnaces.

It will be observed that we have invented a flux free lining and a convenient and wholly satisfactory method and apparatus for heat 5 treating the refractory lining of any type of furnace and which may be used for heat treating other refractory vessels, such as ladies, launders, spouts, etc., which require some kind of refractory lining. Linings so prepared and treated 10 show pronounced economies and advantages in furnace operation. By our invention, not only can new linings be satisfactorily treated, but repairs can be expeditiously made to defective linings. Furthermore, the desirable refractory material 15 may be burned in or fused without the use of fluxes, thus retaining unimpaired the maximum refractory and other desirable qualities of the lining.

While we have illustrated and described certain preferred embodiments of our invention, it will be understood that the invention is not limited thereto and that various changes in the shape, size and arrangement of parts may be resorted to without departing from the spirit of 25 our invention or the scope of the following claims.

We claim:

1. The process of heat treating the refractory lining of a furnace or like structure, which consists in subjecting a limited area of said lining to the action of a mobile electric arc blown 30 against it and thereafter subjecting other areas of the lining to the action of the electric arc until the desired area of the lining has been 35 treated.

2. The process of preparing furnace linings for use which comprises applying and shaping lining material to the interior of a furnace chamber of the ultimate desired contour and thickness and 40 thereafter burning in the shaped refractory by progressively subjecting successive small areas of the lining to the fusing action of an electric arc projected against the surface of the lining.

WILLIAM E. MOORE. 45  
WILLIAM B. WALLIS.